

## UNITED STATES PATENT OFFICE.

CHESTER C. TREISCHEL, OF SCHENECTADY, NEW YORK, ASSIGNOR TO GENERAL ELECTRIC COMPANY, A CORPORATION OF NEW YORK.

## PORCELAIN.

No Drawing.

Application filed June 8, 1921. Serial No. 476,084.

To all whom it may concern:

Be it known that I, CHESTER C. TREISCHEL, a citizen of the United States, residing at Schenectady, in the county of Schenectady, State of New York, have invented certain new and useful Improvements in Porcelain, of which the following is a specification.

The present invention comprises an improved ceramic material, which is particularly useful as a high tension electrical insulator.

Porcelain commonly consists of a mixture of clay, silica and feldspar. I have discovered that the mechanical and electrical insulating properties of porcelain may be markedly improved by introducing certain fluxing silicates into the porcelain other than feldspar, such for example, as the mineral beryl. This material may be substituted totally or in part for either the usual feldspar or silica content.

The percentage of fluxing silicate may vary materially. I have obtained good results with percentages of beryl ranging from five to thirty-five per cent.

The following green or unfired mixture constitutes an example of my invention as embodied in a porcelain suitable for electrical line insulators.

|               |            |
|---------------|------------|
| Clay-----     | 291 parts. |
| Silica-----   | 35 parts.  |
| Feldspar----- | 144 parts. |
| Beryl-----    | 130 parts. |

This mixture is subjected to the usual treatment accorded to porcelain mixtures and finally fired in the usual way to a temperature corresponding to Segar cone 10.

Porcelain having the above composition shows upon test the following improvement over first quality electrical porcelain.

|                                        | Approximate improvement—Per cent. |
|----------------------------------------|-----------------------------------|
| Dielectric strength-----               | 16.5                              |
| Transverse-----                        | 22.5                              |
| Resistance to impact-----              | 44.0                              |
| Resistance to temperature changes----- | 132.0                             |

What I claim as new and desire to secure by Letters Patent of the United States, is:

1. A raw batch for a porcelain mix comprising beryl as a component.
2. A porcelain comprising a fired mixture of clay, silica, feldspar and beryl.
3. An electric insulating material comprising a fired mixture of approximately 291 parts of clay, 35 parts of silica, 144 parts of feldspar and 130 parts of beryl.

In witness whereof, I have hereunto set my hand this 7th day of June 1921.

CHESTER C. TREISCHEL.